

# United States Patent Office

3,194,627

Patented July 13, 1965

1

3,194,627  
PROCESSES FOR PRODUCING MODIFIED  
CELLULOSIC TEXTILE MATERIALS

Dmitry Michael Gagarine, Pendleton, S.C., assignor to  
Deering Milliken Research Corporation, Pendleton,  
S.C., a corporation of Delaware  
No Drawing. Filed Aug. 7, 1958, Ser. No. 753,620  
17 Claims. (Cl. 8—116)

This invention relates to improved methods for producing cellulosic textile materials having minimum-care or flat-drying characteristics, and more particularly the invention relates to methods for producing flat-drying cellulosic textile materials with relatively improved wet strengths. This application is a continuation-in-part of U.S. application S.N. 575,716, filed April 3, 1956, now Patent No. 2,985,501.

According to the disclosure of application S.N. 575,716, now Patent No. 2,985,501, a cellulosic material is impregnated with an aqueous basic solution and reacted with a cross-linking agent under such conditions that the product has a pronounced wet memory and will, when wet, tend to assume the configuration imparted during the cross-linking reaction. It is normally a characteristic of the processes disclosed in application S.N. 575,716, now Patent No. 2,985,501, as well as certain other processes wherein a cellulosic material is reacted with a cross-linking agent in the presence of a base, that the products thereof have, in each instance, a wet tensile strength which is lower than the dry strength of the product and this is disadvantageous for the reason that textile materials produced by these processes are, while wet, frequently subjected to considerable stress during washing.

According to the improved process of this invention, fabrics and yarns having wet strengths approximately equal to their dry strengths are produced by applying to a cellulosic material, in addition to a basic solution and a cross-linking agent, a small quantity of an anti-oxidant material or composition.

It is quite surprising for two reasons that by the simple expedient of applying an antioxidant the wet strengths of textile materials processed according to the above-mentioned procedures can be increased without materially affecting the dry strengths thereof. First, it would normally be assumed that any damages due to oxidation in processes of this type would equally affect the wet and dry strengths and that the unproportional reduction in wet strength could not be due to this cause. Second, the reaction conditions and reagents in these processes are such that no appreciable degree of oxidation damage would be expected and in other processes where a fabric or yarn is impregnated with an alkaline solution under similar conditions, no noticeable degree of oxidation damage is normally encountered. Further, the cross-linking agents employed according to this invention are not known to be oxidizing agents and normally do not act as such. In other words, it is apparently only under the specific conditions present in processes as above described that one experiences, in the absence of an antioxidant, this unusual type of damage which results in a reduction in wet strength without a corresponding reduction in dry strength.

The cross-linking agents which can be employed in the improved process of this invention are those capable of being represented by one of the following formulae:



2



5 wherein X represents halogen; R<sub>1</sub>, R<sub>2</sub>, and R<sub>3</sub> represent, in each instance, a member selected from the group consisting of hydrogen, and monovalent, nonfunctional radicals; R<sub>4</sub>, in each instance, represents a divalent connecting radical; and Z, in each instance, represents a divalent radical selected from the group consisting of those capable of being represented by one of the formulae:



wherein R<sub>5</sub> and R<sub>6</sub>, in each instance, represent hydrogen or a monovalent, nonfunctional radical, and X represents halogen. When a cross-linking compound corresponding to one of the above formulae contains two Z groups, the 20 groups may be the same or different.

R<sub>1</sub>, R<sub>2</sub>, R<sub>3</sub>, R<sub>5</sub>, and R<sub>6</sub> in the above formulae, in each instance, preferably represent hydrogen since such compounds are the most readily prepared, but they can in one or more instances represent lower alkyl groups such as 25 methyl or ethyl; hydroxalkyl groups such as hydromethyl or hydroethyl; monocyclic aryl groups such as phenyl or tolyl; cycloalkyl groups such as cyclohexyl; haloalkyl groups such as chloromethyl and chloroethyl; or R<sub>1</sub> and R<sub>3</sub> can together represent a divalent connecting radical 30 such as a methylene or an ethylene radical. The only requirement is that R<sub>1</sub>, R<sub>2</sub>, R<sub>3</sub>, R<sub>5</sub>, and R<sub>6</sub> must not be such as to prevent the compound from reacting with at least one hydroxy group in two different cellulose molecules.

35 R<sub>4</sub> in the above formulae can represent any divalent connecting group, but in most instances will represent either an alkylene group such as methylene, ethylene, or propylene; a hydroxalkylene group such as hydroxypropylene; or a group of the formula



wherein Y represents oxygen or sulfur, R and R'' represent lower alkylene groups such as methylene or ethylene and R' represents any divalent connecting radical as 45 illustrated by a lower alkylene group, a lower hydroxalkylene group such as 2-hydroxypropylene, a monocyclic aryl radical such as phenylene or tolylene, a radical of the formula —C<sub>2</sub>H<sub>4</sub>(O—C<sub>2</sub>H<sub>4</sub>)<sub>n</sub>— wherein n is an integer of from 1 to about 20; or a radical of the formula



wherein n represents an integer of from 1 to about 5 and R''' represents a divalent hydrocarbon radical as 55 illustrated by



Compounds of the latter type (i.e. containing a



group) result when epichlorohydrin or divinylsulfone is reacted with less than an equal molar quantity of a dihydric alcohol or phenol.

65 The cross-linking agent should in all instances be such that it results in linkages having a chain length of from 3 to 24 carbon atoms and should preferably be such that it results in linkages of from 3 to 10 carbon atoms in length. Specific illustrative examples of suitable cross-70 linking compounds are: epichlorohydrin, 1,3-dichloro-2-propanol, 2,3-dichloro-1-propanol, 2,3-dibromo-1-propanol, m-di(β,γ-epoxypropoxy)benzene, 1,3-di(β-hydroxy-

$\gamma$ -chloropropoxy)-2-propanol, 1,2-di( $\beta$ -hydroxy- $\gamma$ -chloropropoxy) ethane, 1,2-di( $\beta$ , $\gamma$ -epoxypropoxy) ethane, 1,2;3,4-diepoxybutane, 1,2;5,6-diepoxyhexane, 1,5-dihydroxy-2,4-dichloro-cyclohexane and 2,6-dichloro-3,4,5-trihydroxy - 5 - hydroxymethylheptane. The preferred cross-linking compounds are 1,3-dichloro-2-propanol, 2,3-dichloro-1-propanol, and mixtures of the two.

The amount of the cross-linking agent employed may be varied within wide limits under certain conditions, but an amount of the cross-linking agent equal to from about 6% to 30% of the weight of cellulosic fibers is usually satisfactory and from 8% to 15%, by weight of the cellulosic fibers, of the cross-linking agent is preferred. This generally results in the cellulosic fibers gaining from about 2% to 4% in weight.

The basic solution to be employed with the process of this invention can be a solution of any of the well-known strongly basic inorganic or organic materials. Preferably solutions of an alkali metal hydroxide such as sodium hydroxide or potassium hydroxide are employed, but solutions of other bases such as sodium silicate, and quaternary ammonium bases such as trimethylphenylammonium hydroxide and tetramethylammonium hydroxide can also be used. The amount of the basic solution employed should generally be sufficient to provide an amount of water in the fabric equal to from 15% to 130% of dry fabric or yarn weight and preferably from 60% to 90% of dry fabric or yarn weight, and the effective concentration of the basic solution in the fabric or yarn should be from about 3% to 30% and preferably from 5% to 15% by weight.

The process of this invention for forming flat-drying textile materials can be satisfactorily performed with yarns or fabrics containing either natural cellulose fibers, regenerated cellulose fibers, or modified cellulose fibers having a portion of the hydroxy groups therein blocked by ester or ether groups. Examples of materials of the latter type which can be employed include yarns or fabrics composed of cellulose acetate, cellulose butyrate, ethyl cellulose or methyl cellulose fibers. Generally, the cellulosic fibers should have an average of at least about 1.8 free hydroxy groups per glucose unit, and cellulosic materials having a smaller number of free hydroxy groups do not normally give satisfactory results, even though, in the case of cellulose esters, the ester groups might theoretically be removed by hydrolysis during the cross-linking reaction. While the invention is operable with yarns and fabrics formed from cellulose derivatives as above described, it finds its greatest utility with fibers and fabrics formed of unmodified cellulose and particularly with cotton materials.

Satisfactory results, according to this invention, can also be achieved with yarns or fabrics partially composed of other than cellulosic materials, and this is particularly true if the non-cellulosic fibers have some flat-drying properties of their own. For example, the flat-drying tendencies of a yarn spun from a mixture of glycol-terephthalate fibers and cotton fibers can be readily increased by the process of this invention, even if the percentage of cotton fibers is as small as, for example, 10%. Even when the non-cellulosic fibers display no flat-drying properties, yarns or fabrics containing the same can be caused to display flat-drying properties by the new process, if the yarns or fabrics contain at least about 40% by weight of cellulosic fibers.

Almost any antioxidant or mixture of antioxidants can be employed in the improved process of this invention and the antioxidant may be either organic or inorganic in nature. Suitable examples of inorganic antioxidants include readily oxidizable salts such as sodium sulfite, sodium thiosulfate, and sodium sulfide. Examples of suitable organic antioxidants which can be employed include metal formaldehyde sulfoxilates, such as sodium formaldehyde sulfoxilate and zinc formaldehyde sulfoxilate; aldehydes, such as glucose; aromatic alcohols, such as

hydroquinone and pyrogallol; aromatic amines, such as aniline; aliphatic amines, such as octadecylamine; and condensation products of amines and aldehydes, such as the condensation product of aniline and croton aldehyde. Sodium sulfite is generally the preferred antioxidant for use according to this invention for the reasons, among others that it is inexpensive, is readily soluble in basic solutions, and does not discolor in the process.

The amount of the antioxidant employed can be varied within reasonably wide limits, but as a general rule the amount employed should be equal to at least about 0.005% of the weight of basic solution with which the cellulosic material is impregnated and in most instances better results are achieved if the amount of antioxidant material is at least 0.01% of the weight of basic solution. A considerable excess over the minimum required can be employed, but in most instances the nature of the cross-linking agent is such that a reaction with the antioxidant is possible and the use of large excesses of the antioxidant should be avoided. For this and other reasons it is seldom if ever advantageous to employ more than about 8% of the antioxidant, based upon the weight of the basic solution, and in most instances no improvement is obtained by employing more than 3.0% of the antioxidant material.

The cross-linking agent and basic solution may be applied in any suitable manner as illustrated by padding, spraying, brushing or the like. If the basic solution is to be applied first to either a wet or dry textile material, best results are usually obtained by immersing the fabric or yarn in a solution of the base and thereafter passing the textile material through squeeze rolls to remove excess liquid. If the base is to be applied subsequent to the cross-linking agent, it is generally advantageous to apply the same by means of an applicator roll or, in other words, by passing the textile material into contact with a portion of the surface of a roll having another portion of its surface in contact with a supply of the solution to be applied. This eliminates the possibility that a large percentage of the cross-linking agent might be leached from the textile material and results in less hydrolysis of the cross-linking agent that might be obtained by dipping the fabric or yarn into a large volume of the basic solution. The cross-linking agent is in almost all instances best applied by means of an applicator roll because of the relatively small quantity of the agent which need be employed and because this method of application generally results in greater uniformity than spraying.

The most advantageous procedure for applying the antioxidant material to the yarn or fabric comprises adding the same to the basic solution with which the fabric or yarn is to be impregnated, since such a procedure adds no additional manipulative steps to the process, insures that the antioxidant material is present at all times while the fabric or yarn is in contact with the basic solution and insures an even distribution of the antioxidant material. The antioxidant can, however, be applied by padding the fabric or yarn through a solution of the antioxidant or by spraying a solution of the antioxidant onto the fabric or yarn prior to the time that it is impregnated with the alkaline solution. When the cross-linking agent is applied to the textile material prior to the application of the basic solution it may be advantageous to apply an antioxidant with the cross-linking agent, and this is sometimes true even though an antioxidant is also applied with the basic solution. In applying an antioxidant with the cross-linking agent, the most convenient procedure comprises dissolving the antioxidant in the reagent, but it will be understood that this requires the use of an antioxidant which is soluble in the particular cross-linking agent being applied to the cellulosic material.

The cross-linking reaction tends to permanently fix the configuration of the fabric or yarn as that prevailing during the reaction. In other words, if one desires a

fabric that will have a flat and pressed appearance after washing, it is necessary that the fabric be retained in a flat condition during the cross-linking reaction. This can be accomplished by conducting the reaction while the fabric is in a tenter frame or by rolling the same into a tight roll. If desired, the roll of fabric can be wrapped in a water impervious cover, such as aluminum foil or a sheet of vinyl plastic, as illustrated by polyethylene plastic. Of course, if it is desired that the fabric display permanent pleats or the like, then it is necessary that the cross-linking reaction be conducted while the fabric is in a pleated condition.

The cross-linking reaction may be conducted at any suitable temperature below about 110° C. or the boiling point of the basic aqueous solution at the particular pressure under which the reaction is conducted, but for reasons of convenience, the reaction is preferably carried out at room temperature or the temperature naturally resulting from the reaction. The cross-linking reaction is slightly exothermic and, in most instances, will cause a gradual rise in temperature as the reaction progresses, but this is not generally detrimental and no means for retaining the reaction temperature at a constant level are generally necessary. The time required for the cross-linking reaction will vary somewhat with the temperature, the cross-linking agent employed and the order in which the reagents are applied, but even at low temperatures, i.e. 20° C. to 30° C., good flat-drying properties are normally obtained in 24 hours or less, and at 75° C., the reaction is, as a rule, reasonably complete in 20 minutes or less. Exceedingly long reaction times, for example, forty-eight hours or more, can be employed, but the cross-linking reaction is preferably allowed to continue for only so long as is necessary to obtain satisfactory flat-drying properties.

The invention will now be more specifically illustrated by the following examples in which all parts are by weight unless otherwise indicated:

#### Example I

A length of cotton sheeting previously singed, desized, bleached, and frame dried is passed into a solution of 14% sodium hydroxide and squeezed to remove excess liquid so that the total pick-up of sodium hydroxide solution is approximately 90% of the dry weight of the fabric. The alkaline fabric is then passed over an applicator roll by means of which there is applied 11%, based on the dry fabric weight, of a mixture of 1,3-dichloropropanol-2, and 2,3-dichloropropanol-1 in approximately equal parts by weight, and the fabric is thereafter rolled into a tight roll and allowed to remain for approximately 10 hours. The fabric is then unrolled, washed to remove unreacted reagents and dried.

A fabric processed according to this example was found to have a dry tensile strength of 32.7 pounds warpwise and 26.5 pounds fillingwise and a wet tensile strength of 23 pounds warpwise and 18 pounds fillingwise.

#### Example II

Example I is repeated except that to the alkali solution there is added 0.05%, based on the weight of solution, of anhydrous sodium sulfite.

A sample of fabric processed according to the procedure of this example was found to have a dry tensile strength of 33 pounds warpwise and 26 pounds fillingwise and a wet tensile strength of 28 pounds warpwise and 22 pounds fillingwise so that there was more than a 20% improvement in both warp and filling wet tensile strength as compared to the results obtained in the procedure of Example I.

#### Example III

Example II is repeated except that an equal weight of sodium thiosulfate is substituted for the sodium sulfite employed in that example. The results are substan-

tially the same as are obtained by the procedure of Example II.

The procedure is the same as illustrated in the above examples when employing other cross-linking agents, bases, antioxidants and types of textile materials.

Having thus described my invention and two specific embodiments thereof, what I desire to claim and secure by Letters Patent is:

1. In a process for imparting flat drying characteristics to a textile material containing cellulosic fibers having an average of at least about 1.8 free hydroxyl groups per glucose unit, wherein said fibers are reacted with a cellulose cross-linking agent in the presence of a base solution, the conditions of this reaction being such that the wet tensile strength of the fibers is reduced below the dry strength of the fibers, the improvement which comprises applying to said textile material up to about 8% by weight of the base solution of an antioxidant selected from a group consisting of oxidizable inorganic salts, metal formaldehyde sulfoxylates, aldehydes, aromatic alcohols, aromatic amines, aliphatic amines, and condensation products of amines and aldehydes, and retaining said antioxidant on said textile material during the cross-linking reaction whereby the wet tensile strength of the fibers is not reduced to the same extent as would occur in the cross-linking reaction in the absence of said antioxidant.
2. A process according to claim 1 wherein said cross-linking agent comprises divinyl sulfone.
3. A process according to claim 1 wherein said cross-linking agent comprises 1,3-dichloropropanol-2.
4. A process of claim 3 where the base comprises sodium hydroxide.
5. A process of claim 4 wherein the effective concentration of the basic solution in the textile material is from about 3 to about 30% by weight.
6. An improved process according to claim 1 wherein said antioxidant is a readily oxidizable inorganic salt.
7. A process according to claim 6 wherein said antioxidant is dissolved in an aqueous solution of said base and applied simultaneously with said base to said textile material.
8. A process according to claim 7 wherein the amount of said antioxidant added to said basic solution is from 0.01% to 3% by weight of said solution.
9. A process according to claim 8 wherein said antioxidant is sodium sulfite.
10. A process according to claim 8 wherein said antioxidant is sodium thiosulfate.
11. A process according to claim 9 wherein said base is sodium hydroxide.
12. A process according to claim 11 wherein said cross-linking agent is a mixture of dichloropropanols.
13. A process according to claim 12 wherein said textile material is a cotton fabric.
14. In a process for imparting flat drying properties to a textile fabric containing at least about 40% by weight of cellulosic fibers having an average of at least about 1.8 free hydroxyl groups per glucose unit, and wherein said textile material is impregnated with a solution of an alkali metal hydroxide and has distributed thereon a quantity sufficient to result in said cellulose fibers gaining from about 2% to 4% in weight, of a cross-linking agent which results in cross-linkages of from 3 to 10 carbon atoms in length under conditions whereby the wet tensile strength of the fibers is reduced below the dry tensile strength of the fibers, the improvement which comprises applying to said fabric up to about 8%, by weight of the solution of an alkali metal hydroxide, of an antioxidant selected from the group consisting of oxidizable inorganic salts, metal formaldehyde sulfoxylate, aldehydes, aromatic alcohols, aromatic amines, aliphatic amines and condensation products of amines and aldehydes, and retaining said antioxidant on said fabric during the cross-linking reaction.

ing the cross-linking reaction, whereby at least the wet tensile strength of the fibers is considerably improved over the wet tensile strength of fibers similarly treated but in the absence of said antioxidant.

15. A process according to claim 14 wherein said antioxidant comprises sodium sulfite and is applied by being dissolved in said alkali metal hydroxide solution, and is applied in an amount equal to from 0.01% to 0.3% by weight of said alkali metal hydroxide solution.

16. An improved method for imparting a pronounced wet memory to textile materials such as fabrics and yarns containing cellulosic fibers having an average of at least about 1.8 free hydroxyl groups per unit which comprises distributing in and on said textile material water, an alkali metal hydroxide, an anti-oxidant selected from the group consisting of oxidizable inorganic salts, metal formaldehyde sulfoxylates, aldehydes, aromatic alcohols, aromatic amines, aliphatic amines and condensation products of amines and aldehydes, and a cellulose cross-linking agent such that said textile material contains a total amount of water equal to from about 20% to 130% of the dry weight of said cellulose, an amount of alkali metal hydroxide equal to from about 5% to 30% of the total water present, an amount of anti-oxidant equal to from about 0.005% to 3.0% of the total amount of water present, and an amount of said cross-linking agent equal to from 3% to 30% of the dry weight of said cellulose, conforming said textile material, immediately following the distribution of reagents thereon, to a selected configuration, enclosing said textile material to prevent loss of reagents, retaining said enclosed material in said configuration until said cellulose has gained from about 1% to 4% in weight as a result of chemical modification, and thereafter washing said textile material to remove unreacted reagents.

17. An improved method for imparting a pronounced wet memory to textile materials, such as fabrics and yarns, containing cellulose fibers having an average of at least about 1.8 free hydroxyl groups per glucose unit which comprises distributing in and on said textile material water, sodium hydroxide, sodium sulfite, and a mixture of 1,3-dichloro-2-propanol and 2,3-dichloro-1-

30 propanol such that said textile material contains a total amount of water equal to from 20% to 130% of the dry weight of said cellulose, an amount of sodium hydroxide in excess of that required to neutralize the hydrogen chloride eliminated from said dichloro-propanols and equal to from 5% to 15% of the total water present, an amount of sodium sulfite equal to from 0.01% to 1% of the total water present, and an amount of said dichloro-propanols equal to from 3% to 30% of the dry weight of said cellulose, conforming said textile material, immediately following the distribution of reagents thereon, to a selected configuration, enclosing said textile material to prevent loss of reagents, retaining said enclosed material in said selected configuration until said cellulose has gained from about 1% to 4% in weight as a result of chemical modification, and thereafter washing said textile material to remove unreacted reagents.

#### References Cited by the Examiner

##### UNITED STATES PATENTS

|           |       |                  |       |          |
|-----------|-------|------------------|-------|----------|
| 1,392,833 | 10/21 | Jones            | ----- | 8—133    |
| 1,863,208 | 6/32  | Schorger         |       |          |
| 2,157,530 | 5/39  | Ellsworth et al. | ----- | 26—231   |
| 2,181,264 | 11/39 | Dreyfus          | ----- | 8—120 XR |
| 2,524,399 | 10/50 | Schoene          | ----- | 8—116    |
| 2,985,501 | 5/61  | Gagarine         | ----- | 8—120    |

##### FOREIGN PATENTS

|         |      |                |
|---------|------|----------------|
| 291,474 | 6/28 | Great Britain. |
| 531,698 | 1/41 | Great Britain. |
| 696,282 | 8/53 | Great Britain. |
| 724,096 | 2/55 | Great Britain. |

##### OTHER REFERENCES

Marsh, John T.: Mercerising, 1942, pp. 244—247.  
Mercerisation, editors of "The Dyer and Calico Printer," 1903, pages 140—143.

40 NORMAN G. TORCHIN, *Primary Examiner.*

MORRIS O. WOLK, A. LOUIS MONACELL,  
*Examiners.*